

Oct. 26, 1937.

H. DREYFUS

2,096,795

MANUFACTURE OF SPUN YARNS FROM CONTINUOUS FILAMENTS

Filed Nov. 1, 1933



Inventor:  
Henry Dreyfus  
by,  
Geltzer and Dreyfus  
Attorneys

## UNITED STATES PATENT OFFICE

2,096,795

MANUFACTURE OF SPUN YARNS FROM  
CONTINUOUS FILAMENTS

Henry Dreyfus, London, England

Application November 1, 1933, Serial No. 696,183  
In Great Britain November 12, 1932

## 10 Claims.

(Cl. 19—1)

This invention relates to the conversion of continuous filament yarns into yarns having the appearance of spun yarn, that is yarn made by spinning staple fibre.

5 In the manufacture of spun yarn from artificial fibres, the usual practice is to cut continuous artificial filaments or waste filaments into comparatively short lengths, for example of 1½ to 2 inches or more to produce a staple of 10 similar length to cotton fibres, or of 4, 7, 9, 12 inches or more to produce a staple somewhat similar in length to wool, and then subject the 15 staple fibres produced along or mixed with other natural or artificial fibres of suitable length to a series of operations appropriate to the length of the fibre, such operations being similar to those according to natural fibres such as cotton or wool, including opening, carding, drawing and spinning. These operations represent considerable 20 expense in the production of such yarns, since they involve a relatively slow transformation of the initial fibrous material to a finished 25 yarn.

The object of the present invention is to produce 25 yarn having an appearance similar to that of yarn made by spinning staple fibres while avoiding the necessity for forming continuous filaments into short lengths and subjecting the fibres thus produced to a spinning operation. 30 In particular the purpose of the invention is to transform continuous filaments directly into spun yarn by breaking the filaments into staple lengths in the absence, however, of the considerable reduction in extensibility which ordinarily results from the stretching of filaments to 35 breaking point.

Broadly, the invention contemplates rendering the filamentous material brittle in character, so that under the application of a stretching 40 load breakage occurs with little or no extension of the filaments. Breaking thus taking place with little or no extension, the filaments are not subjected to internal strain which results in loss in extensibility, and the spun yarn produced 45 from these filaments has thus sufficient elasticity to enable it to be manipulated satisfactorily in textile operations.

The invention is particularly important in connection with the conversion of filaments of cellulose acetate or other cellulose derivatives, for 50 example cellulose esters such as cellulose formate, propionate, and butyrate, and cellulose ethers such as ethyl, methyl and benzyl cellulose, but may be generally applied for the conversion 55 of filaments into staple fibres. For example, in

operating on filaments of cellulose acetate or other thermoplastic cellulose derivative, the temperature of the filaments may be so lowered that they become more rigid, and so capable of being broken with little extension. It is, however, advantageous to make use of the moisture or other liquid which textile materials are capable of absorbing to a greater or lesser degree, since the freezing or solidifying of included liquid has the effect of imparting brittleness even if the material of the filaments has not reached that state. If necessary, the filaments may be specially conditioned before exposing them to the refrigerating medium in order to bring them into a state in which they can be easily broken without the use of very low temperatures. The invention enables breakage to be effected with the application of comparatively small load in machines of relatively light construction.

Quite low temperatures may be employed in carrying out the invention, e. g. down to  $-80^{\circ}$  C. and for this purpose liquid gas, for example liquid air may be employed.

While liquid air has been mentioned as an example of suitable cooling medium, it will be understood that any other liquid or gaseous medium may be employed which is capable of bringing the filaments to the requisite low temperature. Thus, cooled brine may be used as a medium to bring the filaments to such a degree of brittleness as materially to reduce loss of extensibility on breakage. Good results are obtained with cellulose acetate filaments cooled to about  $-5^{\circ}$  C.

In view of the brittle nature of the filaments, it is desirable that the gripping devices themselves should not be such as to produce a rupture of the filaments merely by contact of the devices with the filaments. Pairs of rollers rotating at different speeds and spaced apart at a distance corresponding to the length of staple to be produced form convenient gripping means to exert the desired breaking action on the filaments.

In order to avoid danger of further filament breakage after the filaments have been transformed into staple fibres of the desired length by the gripping devices, means may be provided to restore the filaments rapidly to their original condition. For example, filaments rendered brittle by cooling as described above may be withdrawn from a cooled chamber in which they are broken and given atmospheric temperature by contact with the air, or they may even be passed over heating means or jets of hot air

immediately after breakage. The broken filaments then form a coherent mass capable of being delivered to a twisting device which imparts twist and strength to the fibrous yarn. By twisting continuously with breaking uniformity of the fibre distribution is maintained, with consequent advantage to the quality of the product. A twist tube or like device may be employed to impart false twist to the material leaving the breaking device, so as to give it sufficient strength to maintain itself until a definite degree has been imparted by the flyer of the twisting spindle. If required supporting means may be provided between the rollers of the breaking device, such means conveniently comprising an endless band or pair of bands driven at an appropriate linear speed.

Any desired number of yarns may be converted into fibres in a single breaking apparatus. Several filamentous yarns may be led side by side to the apparatus and the fibres of these several threads may either be drawn together into a single sliver or may be maintained separate and separately twisted into a roving on leaving the apparatus. Thus, one such apparatus may serve a plurality of twisting spindles.

After breakage, the fibrous bundle may be passed directly through draw rollers to reduce the size of the bundle, in which case the final yarn 30 may be produced in the one continuous operation. If desired, a ring-spinning device may be used to impart the relatively high degree of twist in such final product. Two or more twisted yarns may be doubled together at any drawing stage to increase the evenness and strength of the final yarn.

Forms of apparatus suitable for carrying out the process according to the invention will now be described with reference to the accompanying drawing, in which:—

40 Fig. 1 shows in end elevation, filament cooling and breaking apparatus, certain frame elements being omitted for the sake of clarity.

Fig. 2 is a part sectional plan view of the apparatus shown in Fig. 1, while Fig. 3 shows somewhat diagrammatically in end elevation another form of apparatus.

As shown in Figs. 1 and 2, continuous filamentary bundles 5.5, preferably in untwisted form, unwinding from packages 6.6, are led through guides 7.7 and eventually to bobbins 8.8 of flyer-spinning devices 9.9. After leaving the guides 7.7 the bundles pass through the nip of rolls 10, 11 the roll 11 being disposed in such a manner that the bundles contact with a relatively 55 large part of the periphery of the roll 10, the extent of the arc of contact being indicated in dotted lines.

The lower roll 10 is hollow and is connected by a supply pipe 12 and an exhaust pipe 13 to a refrigerant supply, (not shown) from which refrigerant, e. g. brine, is passed through the roll as indicated by the arrows. Each pipe joint is maintained tight and comprises a nut 14 which screws on to a threaded hollow extension 15 of the roll 65 axle and urges a circumferential lug 16 of the pipe against a packing 17 which is compressed against the extension 15 and tends to expand outwardly against the inner wall of the nut 14. The roll 10 is thus free to rotate while the pipes 12 and 13 are stationary, and no refrigerant is lost.

The upper roll 11 is maintained at low temperature by reason of its close proximity to the cooled lower roll 10, and is supported in suitable bearings in arms 18, to be described later. On passing 75 between the cooled rolls, the bundles 5.5 are re-

duced to very low temperature and thus rendered brittle prior to passing through the nips of two pairs of rolls 19, 20 and 21, 22, the latter pair of which rotate at a higher rate than 19, 20, and break the filaments comprising the bundles into lengths substantially equal to the "ratch" or distance between the axes of the rolls 19, 21. The brittle nature of the filaments renders considerable pressure on the nip rolls unnecessary, and the weight of the upper rolls may be sufficient to cause firm gripping of the bundles.

The fibrous nature of the ruptured bundles generally maintains their continuity, but if desired, supporting means such as a travelling endless band or carriers may be arranged beneath the bundles between the rolls 19, 20 and 21, 22. The bundles 5.5 are delivered from the rolls 21, 22 in the form of untwisted fibrous sliver and proceed to the flyer-spinning devices 9, over guides 23.23 where they are relatively lightly twisted and wound on the bobbins 8.8.

The cooling and breaking rolls may be of any desired length, necks being formed at suitable intervals to provide bearing surfaces for supporting means. Thus while four bundles only are shown in the figures, as many bundles as desired may be processed simultaneously merely by lengthening the rolls in accordance with the number of bundles to be treated.

The upper rolls 11, 20 and 22 are preferably quickly and simultaneously removable in order to allow of rapid forwarding by hand of new or broken bundles. This is effected conveniently by bearing the bosses of all the upper rolls, viz. 11, 20, and 22, in the arms 18 and pivoting the arms 35 to the roll-supporting frame 24 at points 25.25. Thus, on lifting the arms 18, 18, the upper rolls are removed from contact with the lower rolls and leave room for bundle manipulation between the two sets. Conveniently, short lengths only of the 40 upper rolls extend between successive pairs of arms 18, 18 so that on lifting the arms, the processing of the minimum possible number of bundles is interrupted. Where such interruption is of frequent occurrence, it is advisable to mount 45 sets of upper rolls singly, the lower rolls extending, of course, along the whole length of the machine in uninterrupted order.

If it is desired to impart to the bundles 5.5 a greater degree of brittleness for a given low temperature, they may be passed over and in contact with wicks 26.26 supplied with moisture from a trough or pipe 28 placed between the guides 7.7 and the roll 10, so that the bundles are dampened before passing between the cooling rolls. The 55 moisture thus applied to the bundles freezes on the filaments on contacting with the rolls 10, 11 and enables them to be more easily broken.

In order to remove the frozen moisture so formed, and to restore the original temperature 60 and pliability to the filaments after the breaking operation, hot air from a jet 27 may be directed at the bundles, or at each bundle, during the passage from the rolls 21, 22 to the flyer-spinning device. While each bundle is shown proceeding to a separate flyer device, two or more bundles (now, of course, in the fibrous state) may be united and doubled together as a thick sliver or roving after leaving the rolls 21, 22, and led to a common flyer device, or, instead of leading the 70 roving directly to a flyer device, the roving may be drafted to a finer count and then spun into thread.

Alternatively or in addition to the above mentioned cooling method, cooling pipes may be run 75

through the space enclosed by the frame-work 24 immediately beneath the rollers, thus maintaining the whole apparatus at low temperature.

According to the apparatus shown in Fig. 3 5 the cooling means are not removed from the breaking means, the lower rear roll 30 of a breaking-roll set 30, 31 and 32, 33 itself serving to effect the required cooling. The roll 30 is hollow and is supplied with refrigerant in a manner similar 10 to that shown with reference to the roll 10 of Figs. 1 and 2.

The bundles 34 after being cooled and ruptured into masses of fibres between the rolls 30, 31 and 15 32, 33 pass to drawing rolls 34, 35 and 36, 37, maintained under pressure by a bridge 40 tightened by a nut 42 and bolt 41, where the masses 20 of fibres are drawn and reduced in cross section to a sliver, the fineness of which depends on the rate of rotation of the rolls 36, 37 relative to the rolls 34, 35. The drafted slivers so produced may be led singly through balloon guides 39 to a 25 ring-spinning device 43 (one shown) where they are directly twisted into finished threads, or two or more slivers may be united and twisted together into thread by a single ring-spinning device. Drawing continuously with the breaking operation thus enables finished threads to be produced continuously in a single operation.

The moisture-applying device 26 of Fig. 1 may 30 be incorporated in the apparatus of Fig. 3, and hot air blasts may be directed at the material after the breaking operation, so as to remove the imparted brittleness at least in part, and bring the fibres into substantially the same condition as the 35 filaments before being subjected to the cooling operation.

What I claim and desire to secure by Letters Patent is:—

1. Process for the production of staple fibre 40 from continuous filaments, which comprises cooling the filaments to such a temperature as to render them temporarily brittle and while they are in a brittle condition breaking them into short lengths whereby the extensibility of the 45 filaments is substantially preserved.

2. In a process for the production of staple fibre, 50 yarns from continuous filaments, the successive steps of cooling a plurality of continuous filaments to such a temperature as to render them temporarily brittle, and subjecting the brittle filaments to a breaking load so as to break said filaments at different points along their length and transform them into a continuous bundle of staple fibres whereby the extensibility of the filaments 55 is substantially preserved.

3. In a process for the production of staple fibre 60 yarns from continuous filaments, the successive steps of moistening and cooling a plurality of continuous filaments so as to render them temporarily brittle, and subjecting the brittle filaments to a breaking load so as to break said filaments at different points along their length and transform them into a continuous bundle of staple fibres.

4. In a process for the production of staple fibre 65 yarns from continuous filaments, the successive steps of applying moisture to a plurality of continuous filaments, cooling said moistened filaments so as to freeze said applied moisture 70 and subjecting the filaments thus rendered brittle to a breaking load so as to break said filaments

at different points along their length and transform them into a continuous bundle of staple fibre.

5. In a process for the production of staple fibre 5 yarns from continuous filaments, the successive steps of rendering temporarily brittle a plurality of continuous filaments by cooling the same, subjecting the brittle filaments to a breaking load so as to break said filaments at different points along their length and transform them into a 10 continuous bundle of staple fibres whereby the extensibility of the filaments is substantially preserved, and twisting and winding said bundle.

6. In a process for the production of staple fibre 15 yarns from continuous filaments, the successive steps of rendering temporarily brittle a bundle of continuous filaments by cooling the same, subjecting the brittle filaments to a breaking load so as to break said filaments at different points along their length and transform them 20 into a continuous bundle of staple fibres whereby the extensibility of the filaments is substantially preserved, drafting said bundle and spinning the drafted fibres into yarn.

7. In a process for the production of staple fibre 25 yarns from continuous filaments, the successive steps of cooling a plurality of continuous filaments to such a temperature as to render them temporarily brittle, subjecting the brittle filaments to a breaking load so as to break said 30 filaments at different points along their length and transform them into a continuous bundle of staple fibres whereby the extensibility of the filaments is substantially preserved, and applying heat to said filaments to restore them to a non- 35 brittle condition.

8. In a process for the production of staple fibre 40 yarns from continuous filaments, the successive steps of rendering temporarily brittle a plurality of continuous filaments of cellulose acetate or 45 other organic derivative of cellulose by cooling the same, and subjecting the brittle filaments to a breaking load so as to break said filaments at different points along their length and transform them into a continuous bundle of staple fibres whereby the extensibility of the filaments is substantially preserved.

9. In a process for the production of staple fibre 50 yarns from continuous filaments, the successive steps of bringing a plurality of continuous filaments of cellulose acetate to a temperature of about  $-5^{\circ}$  C. so as to render the filaments temporarily brittle, and subjecting the brittle filaments to a breaking load so as to break said filaments at different points along their length and 55 transform them into a continuous bundle of staple fibres whereby the extensibility of the filaments is substantially preserved.

10. In a process for the production of staple fibre 60 yarns from continuous filaments, the successive steps of rendering temporarily brittle a plurality of continuous filaments by cooling the same, and subjecting the brittle filaments to a breaking load so as to break said filaments at different points along their length and transform 65 them into a continuous bundle of staple fibres whereby the extensibility of the filaments is substantially preserved, and blowing heated gas on to the fibres to restore them to a non-brittle condition.

HENRY DREYFUS.